

# UNITED STATES PATENT OFFICE.

MAURICE N. AISEN, OF CHICAGO, ILLINOIS.

## SIZING SOLUTION AND METHOD OF MAKING THE SAME.

1,224,125.

Specification of Letters Patent.

Patented May 1, 1917.

No Drawing.

Application filed April 28, 1914. Serial No. 834,884.

### To all whom it may concern:

Be it known that I, MAURICE N. AISEN, a subject of the King of Roumania, residing at Chicago, in the county of Cook and State 5 of Illinois, have invented a certain new and useful Sizing Solution and Method of Making the Same, of which the following is a specification.

The universal practice heretofore, so far 10 as known to me, of making sizing has been to dissolve glue or gelatin in water, the solution being prepared by first soaking the glue or gelatin for a few hours in cold water, during which time it will absorb many times 15 its weight of water. To effect solution the mass is heated and stirred, its consistency depending upon the relative proportions of water and glue or gelatin. For the best results the temperature should not exceed 212° 20 F. Such sizing solution is used in several arts, that most familiar to me being the manufacture of hats. In the manufacture of straw braid hats, according to known methods, the hat is formed by stitching a 25 continuous length of braid with an allowance for shrinkage. In sizing a hat of this character it is placed upon a block and the hot sizing rubbed in by a sponge or cloth with which it is applied by hand. The sizing 30 must be kept hot and sufficiently dilute to permit proper working by the operator and absorption by the hat material. The excess of material allowed in the hat for shrinkage is taken up during the application 35 of the sizing and the hat will shrink to the mold or block upon which it must remain until it is dry or has become set, or it may be removed from the mold after the sizing has set into the fiber sufficiently far 40 that there is no liability of further shrinkage. The drying of the hat, either on or off the block, has usually been done in an open room at atmospheric temperature, taking about twelve hours, more or less, according 45 to the degree of humidity of the atmosphere. It has sometimes been done in a heated drying room, but the hat must remain on the mold to prevent excessive shrinkage.

Among the disadvantages due to the use 50 of a water solution of glue, and well known to those familiar with the hat industry, are the expense incident to the number of blocks or molds required, the space required in their use and for their storage, and the relatively high cost, as an operator must size 55 each hat separately, place it upon the block

or mold, apply the sizing and remove it by hand, each hat requiring two or three minutes to complete. The greatest objection, however, is due to the difference in the coefficients of contraction of the braid or other material of which the hat is made, the thread with which the braid is stitched, and the glue or gelatin. Because of this difference, the conditions which give rise to the 60 shrinkage, and those which exist at the time the shrinkage takes place, must be so regulated that the greater contraction of the cotton thread in drying will not distort or wrinkle the braid.

As it is the presence of the water in the sizing which gives rise to the shrinking of the material to which the sizing is applied, the problem has been to retain the use of glue or gelatin as a sizing material, because 65 of its cheapness and effectiveness, and to find some other solvent the use of which would not result in the shrinking of the goods treated. My efforts have, therefore, been directed along this line and I have succeeded in 70 modifying the properties of glue and gelatin by hydrolysis thereby rendering them soluble in an organic solvent such as methyl or ethyl alcohol, such composition when applied to a fabric will not cause the fabric 75 to shrink. Also, it permits the sizing of hats in relatively large numbers at one time, thereby materially reducing the cost connected with the sizing operation.

The chief constituent of all glue, that which 80 in the main imparts to it the property of gelatination, is gelatin, but it is difficult to define the exact point of transition from glue to gelatin, both possessing in common 85 the property of water absorption and subsequent gelatination. Commercially the distinction is based largely upon the appearance of the product. I have, therefore, used the term "glue" as including gelatin, and as meaning animal albuminoids and glues of 90 gelatinic basis, which heretofore, so far as known to me, have been insoluble in alcohol, acetone, ether and other organic solvents. As hydrolyzing agents I have used 95 mineral acids, such as nitric acid, hydrochloric acid and sulfuric acid. Organic acids may be used in connection with a mineral acid and, among others which I have used, are formic acid, acetic acid and lactic acid. Or I may use an alkaline hydrolyzing 100 agent such as potassium or sodium hydroxid. 105 The present application will be confined to 110

the composition of matter itself and a method of making it.

The hydrolysis of the glue and its solution in alcohol may be effected in several ways, 5 among them the following:

Example 1: I take two and one-half pounds of nitric acid 70 per cent. pure, and add one and one-quarter pounds of formic acid 25 per cent. pure, and three and one-half pounds of water. These are mixed and shaken or agitated in any convenient manner to produce a homogeneous mixture. I then add ten pounds of powdered glue and mix, taking care that the glue is well covered by the liquid. This is allowed to stand from one to three hours, and then I add alcohol as desired and shake or agitate for about fifteen minutes.

Example 2: I take about eight to ten pounds of hydrochloric acid, calculated as pure hydrogen chlorid, to 100 pounds of glue, and add the acid to one gallon of alcohol. To this liquid, while heated to about 120° to 130° F., the glue is added and the mixture allowed to stand at that temperature for about one hour with occasional stirring; during this time hydrolysis of the glue ensues and the glue is dissolved in the alcohol. Any suitable means for heating the 30 solution may be provided.

Example 3: The glue may also be dissolved by mixing it, preferably in powdered form, with an aqueous solution of an organic acid, such as formic acid, tannic acid, tar- 35 tatic acid, or the like, and passing through the mixture sulfurous acid gas, hydrochloric acid gas, or like acid forming-gas, introducing the gas into the body of the mixture, which is in a closed tank or vessel, and permitting it to permeate through the same. This produces a viscous liquid of about the consistency of thick syrup to which alcohol is added in sufficient quantity to produce the desired viscosity of the alcoholic solution, 45 the mixture being agitated for about fifteen minutes. In following this mode of producing the solution I add two pounds of formic acid 25 per cent. pure to two pounds of water and shake until thoroughly mixed. 50 I then add ten pounds of powdered glue and mix, taking care that the glue is well covered by the liquid. The mixture is placed in a closed vessel and into it is introduced a current of sulfurous acid gas or hydrochloric acid gas, for a period of from one to two hours, the mixture being maintained at a temperature of from 80° to 90° F. The alcohol is then added as desired and the mass agitated for about fifteen minutes.

Example 4: Ten per cent. of potassium hydroxid, of the weight of glue to be dissolved, is dissolved in two gallons of alcohol and the mixture heated to about 120° F. The glue is then added, with stirring, and the mixture heated to about 145° to 150° F.

in a vessel containing means to recover the alcohol vapor. The mixture is heated at this temperature for about one hour or one hour and a half and then neutralized by the addition of a suitable acid either completely 70 or to any desired degree which is not harmful to the glue or to the material treated.

A certain amount of acid does not render the composition unsuitable for certain industrial purposes. An undue amount of 75 mineral acid will in time impair the efficiency of the composition as a sizing, and if permitted to remain in the composition might hydrolyze the glue to a degree which will render the composition less effective. 80 Also the acid is apt to be harmful to cellulose braids of which hats are made. Therefore, when the composition of examples 1, 2 or 3 is to be used as a sizing I either neutralize all the mineral acid, or neutralize it to a 85 degree at which its presence is not harmful, either to the glue or to the hat material, say down to 1 to 5 per cent. by weight of the acid used. An organic acid, if used, does not destroy or impair the qualities of the 90 glue and need not be neutralized when the compound is used as a sizing. The neutralization of the acid, if such is necessary or desired, may be effected by adding sodium or potassium hydroxid, sodium carbonate or the like. The salts produced by reaction between the neutralizing alkali and the acid are either precipitated, in which case the solution may be filtered or decanted, or will remain in solution in the alcohol 95 without detriment to the sizing.

Instead of using an acid direct, I may use salts which, in their respective water solutions, will develop an acid by hydrolysis, as for example, bisulfite of soda, chlorid of zinc 100 or other salt having the same property.

I have found that the presence of a certain amount of water, even 25 to 30 per cent., in the solution is not detrimental; the amount of water which may be present without detriment depends upon the coefficient of contraction of the goods.

In the method above described in which a mineral acid and an organic acid are mixed in solution, the organic acid increases the stiffness of the sizing on the goods to which it is applied. And in that process in which an acid forming-gas is passed through an organic acid solution the latter serves as a solvent for the former, thereby reducing to 110 some extent the amount of mineral acid required to effect the hydrolysis of the glue.

The composition obtained by any one of the above described methods, that is, a composition of matter containing glue dissolved in alcohol, may be used in ways known in the arts for which sizings are necessary, and I have in a companion application described and claimed a mode of use which has proved beneficial in the hat industry.

What I claim and desire to secure by Letters Patent of the United States is:—

1. As a composition of matter a neutral alcoholic solution of glue.
  - 5 2. As a composition of matter, a neutral alcoholic solution containing glue hydrolyzed by an acid.
  - 10 3. As a new article of manufacture, a neutral alcoholic sizing solution containing glue of gelatinic basis, hydrolyzed by an acid.
  - 15 4. A sizing consisting of a liquid vehicle having non-shrinking tendencies on cellulose material and containing a stiffening substance dissolved in said vehicle.
  5. A sizing consisting of a liquid vehicle having non-shrinking tendencies on cellulose material and containing glue dissolved in said vehicle.
  - 20 6. The method of making a solution containing glue consisting in first hydrolyzing the glue by an acid, then dissolving it in an organic solvent, and then neutralizing the acid to the degree desired.
  - 25 7. The method of making a solution containing glue consisting in first hydrolyzing the glue, then dissolving it in alcohol, and then neutralizing the acid to the degree desired.
  - 30 8. The method of making a solution con-
- taining glue consisting in first hydrolyzing the glue by a mixture of a mineral acid and an organic acid, and then dissolving it in an organic solvent.
9. The method of dissolving glue in alcohol by mixing an acid with the alcohol and then treating the glue with the mixture of acid and alcohol with the application of heat.
10. The method of manufacturing an al- 40 coholic sizing solution consisting in mixing an acid with alcohol, then dissolving glue in the mixture of acid and alcohol with the aid of heat, and then neutralizing the acid in the solution to the degree required. 45
11. The process of manufacturing an alcoholic sizing solution consisting in mixing a mineral acid with alcohol, heating the said mixture and adding glue thereto and maintaining the temperature until the glue is 50 dissolved, and then neutralizing the acid in the solution to the degree required.
- In testimony whereof I have hereunto signed my name in the presence of two subscribing witnesses.

MAURICE N. AISEN.

Witnesses:

E. CALDWELL,  
E. PASCHKE.